

April 26, 1966

C. J. GANCI

3,248,679

METAL ALLOY RESISTORS

Filed Dec. 11, 1962

Fig. 1.



Fig. 2.



Fig. 3.



Fig. 4.



Fig. 5.



INVENTOR.

Charles J. Ganci  
BY

Frank C. Brown  
his ATTORNEY

3,248,679

## METAL ALLOY RESISTORS

Charles J. Ganci, Bellrose Manor, N.Y., assignor to  
Ward Leonard Electric Co., Mount Vernon, N.Y., a  
corporation of New York

Filed Dec. 11, 1962, Ser. No. 243,888  
3 Claims. (Cl. 338—264)

This invention relates to electrical resistors and particularly to the composition of the metal alloy forming the element.

The invention is particularly directed to electrical resistors with wound resistive elements on a ceramic base and covered by a vitreous enamel coating. For good thermal and physical shock qualities, the base of the resistor should have a low coefficient of expansion and the coefficient of expansion of the coating should be slightly lower than that of the base. For high quality, high precision, reliable resistors it is also desirable that the resistance element have certain characteristics and meet certain standards.

Some of these are that the temperature coefficient of resistance should be zero or nearly zero so that the resistor may be subjected to high temperatures in operation without a material or, if possible, any change in resistance value of the resistive element due to temperature rise; and that the alloy should have a ductility and high tensile strength in order to form fine, strong wire or ribbon. The resistance value of the element should remain substantially constant over sustained periods of high heats so as to have a stable electrical load life.

A particularly desirable feature is to have the low coefficient of expansion of the base and the linear coefficient of thermal expansion of the element approximately the same. Heretofore the coefficients of expansion of the resistive elements have been approximately twice that of the base. The coefficient of expansion of the base has been  $6$  to  $9 \times 10^{-6}$  inches per inch per degree centigrade, while that of the resistive elements has been  $15$  to  $18 \times 10^{-6}$  inches per inch per degree centigrade.

When the coefficient of expansion of the wire is substantially greater than the coefficient of expansion of the base, difficulties are encountered during the formation of the protective coating. The resistor is subjected to high temperatures, the wire expands and loosens which causes the wires to pull, bunch or swim, possibly causing shorting of the turns which may result in rejections for resistance values creating hot spots and resulting in unreliability.

Also, the different and lower coefficient of expansion of the coating further aggravates these difficulties.

An object of this invention is to provide an electrical resistor having a base with a low coefficient of expansion and a resistive element of substantially the same coefficient of expansion as the base.

Another object of the invention is to provide a resistance element that has a low temperature coefficient of resistivity and a comparatively low temperature coefficient of expansion that is ductile and has a high tensile strength.

Other and further objects will be apparent from the description taken in connection with the drawings, in which

FIG. 1 illustrates a wire wound tubular resistor with tab type terminals;

FIG. 2 illustrates a wire wound tubular resistor with axial leads;

FIG. 3 illustrates a plaque type of resistor;

FIG. 4 illustrates a strip type of resistor;

FIG. 5 illustrates a disc type of resistor; and

FIG. 6 illustrates a tubular base with a crinkled ribbon type of resistive element.

The base 10 may be made of ceramic or other insulating material for supporting the terminals 11 and 12 and the resistor element 13. The base 10 has a cylindrical

shape and the resistance wire is helically wound on the base and soldered or welded to the terminals 11 and 12. A coating 14 may encase the wire and terminal to protect the wire from physical injury and corrosion. A vitreous enamel coating is illustrated, but other types of coatings, such as cements, Teflon, silicone and the like, may be used depending upon the particular characteristics desired.

The base 10 may be composed of various types of ceramics, such as steatite, alumina, modified talc, fosterite compositions, zircon compositions and other known ceramics. The linear coefficient of thermal expansion of steatite is  $7 \times 10^{-6}$  to  $8.5 \times 10^{-6}$ , fosterite is  $10$  to  $10.5 \times 10^{-6}$  or less, zircon is  $5$  to  $7.5 \times 10^{-6}$  and alumina is  $7$  to  $8.5 \times 10^{-6}$  inches per inch per degree centigrade. Illustrative compositions of these ceramics are set forth as follows:

Table I

|    |                                       | Percent |
|----|---------------------------------------|---------|
| 20 | Zircon:<br>$Zr_5O_4$ (zircon) -----   | 65      |
|    | Plastic clay -----                    | 15      |
|    | Calcium zirconium silicate -----      | 20      |
| 25 | Steatite:<br>Talc -----               | 94      |
|    | Clay -----                            | 4       |
|    | Barium titanate -----                 | 2       |
| 30 | Fosterite:<br>Talc -----              | 75      |
|    | Clay -----                            | 4       |
|    | Barium titanate -----                 | 2       |
|    | MgO -----                             | 19      |
| 35 | Alumina:<br>$Al_2O_3$ (alumina) ----- | 95      |
|    | $SiO_2$ -----                         | .63     |
|    | $CaO, MgO$ -----                      | .63     |
|    | Clay -----                            | 3.75    |

The metal of the terminals 11 and 12 has a coefficient of expansion approximately the same as the ceramic base 10 and may be an alloy, such as a nickel-iron alloy having a range of coefficients from very low to  $16 \times 10^{-6}$  inches per inch per degree centigrade. Alloys having coefficients of expansion in the range of  $6$  to  $10 \times 10^{-6}$  are selected to match the coefficients of expansion of the foregoing ceramic bases. Thus the terminals will have substantially the same or the same coefficient of expansion as the base.

The particular resistive element of this invention comprises a titanium alloy including vanadium and aluminum. Various compositions are set forth as follows:

Table II

|    | A              | B        | C       |
|----|----------------|----------|---------|
|    | Percent        | Percent  | Percent |
| 55 | Vanadium ----- | 13       | 14      |
|    | Chromium ----- | 11       | 11      |
|    | Aluminum ----- | 3        | 3.5     |
|    | Hydrogen ----- | Very low | Low     |
|    | Titanium ----- | 73       | 71.5    |

The linear coefficients of expansion for these alloys are approximately  $9.5$  to  $10 \times 10^{-6}$  inches per inch per degree centigrade. These alloys have a specific resistance of about 900 ohms per circular mil foot and a temperature coefficient of resistivity of less than 100 parts per million.

The alloys have good ductility and tensile strength and may be formed into small diameter wires or thin ribbons. The wires are easily wound on the base in conventional manner and secured to the base by conventional means, such as welding.

Various types of well-known coatings may be used to encase the resistive element and terminals as illustrated. Vitreous enamel coatings should have coefficients of ex-

pansion less than the coefficients of expansion of the base material in order to avoid crazing of the enamel. The coefficients of expansion are in the range of 5 to  $9 \times 10^{-6}$  inches per inch per degree centigrade. Cement, plastic and other types of coatings may be used.

In FIG. 2 the invention is illustrated in connection with an axial type of resistor having end cap 16 mounted on the base 10 with the axial leads 18. In FIG. 3 the wire element is wound in a non-inductive manner on a plaque type of base fragmentarily shown. The wire element 19 is formed on the posts 20 and embedded in a vitreous enamel or cement coating. In FIG. 4 a resistor with an elliptical base 21 is partially illustrated with the tab type of terminal 22 and a wire wound resistive element 23. A vitreous enamel coating is illustrated at 24. FIG. 5 illustrates a radial type of resistor with the resistive element 25 intertwined in bosses 26.

In FIG. 6 a tubular base resistor is illustrated with a crinkled ribbon type of resistive element 27 formed on the base 28 and attached to terminals 29. In referring to a wire type of resistive element, the ribbon form is included in the meaning of this term. The titanium alloy forms a tough ribbon wire which retains its shape and is easily wound on the base.

A preferred form of the base to match coefficients of expansion of the base and the resistance element is a beryllium oxide base of 99 to 100% beryllium oxide. This produces an electrical resistor of greater reliability and higher wattage for a given size. The beryllium oxide base has a very good heat conductivity for conducting the heat of the resistive element.

In addition to the resistive element and the base having substantially the same coefficient of expansion, the terminals may be also made of the metal alloy that has a coefficient of expansion substantially equal to that of the base. The coatings may be any of the well-known coatings as previously mentioned, and if a vitreous enamel coating is used the coefficient of expansion should be slightly less than that of the beryllia base.

I claim:

1. An electrical resistor comprising an insulating core of ceramic composition having a coefficient of expansion between 5 to  $10.5 \times 10^{-6}$  inches per inch per degree centigrade, metal terminals mounted on said core having a coefficient of expansion substantially equal to said core, and a helically formed elongated resistive element of titanium alloy including vanadium and aluminum on said core and in engagement with said metal terminals, said element having a coefficient of expansion of  $9.5$  to  $10 \times 10^{-6}$  inches per inch per degree centigrade.
2. An electrical resistor as set forth in claim 1 wherein the titanium metal alloy comprises 11% chromium, 14% vanadium, 3.5% aluminum and the balance titanium.
3. An electrical resistor as set forth in claim 1 wherein the titanium metal alloy comprises 4% vanadium, 6% aluminum and 90% titanium.

References Cited by the Examiner

UNITED STATES PATENTS

|    |           |         |                |       |            |
|----|-----------|---------|----------------|-------|------------|
| 20 | 2,318,435 | 5/1943  | Stupakoff      | ----- | 174—152.4  |
|    | 2,425,032 | 8/1947  | Deyrup         | ----- | 338—352    |
|    | 2,691,088 | 10/1954 | Ungewiss       | ----- | 338—302    |
|    | 2,696,544 | 12/1954 | Poch           | ----- | 338—302    |
| 25 | 2,697,675 | 12/1954 | Gaiser         | ----- | 338—309 X  |
|    | 2,804,409 | 8/1957  | Kessler et al. | ----- | 75—175.5 X |
|    | 2,864,697 | 12/1958 | Busch et al.   | ----- | 75—175.5 X |
|    | 2,898,570 | 8/1959  | Patrichi       | ----- |            |
| 30 | 2,906,654 | 9/1959  | Abkowitz       | ----- | 75—175.5 X |
|    | 2,940,845 | 6/1960  | Jaffee et al.  | ----- | 75—175.5 X |
|    | 3,147,115 | 9/1964  | Vordahl        | ----- | 75—175.5   |

FOREIGN PATENTS

|    |         |        |                |
|----|---------|--------|----------------|
| 35 | 579,735 | 8/1946 | Great Britain. |
|    | 768,805 | 2/1957 | Great Britain. |

RICHARD M. WOOD, Primary Examiner.

V. Y. MAYEWSKY, Assistant Examiner.